

## UNITED STATES PATENT OFFICE

2,180,697

## LUBRICATING OIL COMPOSITION

Arnold C. Vobach, Whiting, Ind., assignor to  
 Sinclair Refining Company, New York, N. Y.,  
 a corporation of Maine

No Drawing. Application May 17, 1937.  
 Serial No. 143,121

16 Claims. (Cl. 87—9)

My invention relates to improvements in compounded lubricating oils. The improved lubricating oil compositions of my invention consist essentially of a petroleum lubricating oil having dissolved therein one or more metallic aromatic stearates, or metallic aromatic stearates together with metallic stearates, or metallic aromatic stearates or a mixture of metallic aromatic stearates and metallic stearates together with an aromatic stearic acid, stearic acid or palmitic acid. The addition of such soaps or soaps and free acid should be made in amount or amounts insufficient materially to alter the normally liquid character of the petroleum lubricating oil itself, for example, from 0.5% to 2.5% on the oil.

Metallic aromatic stearates, which may be employed with great advantage to produce the improved compounded lubricating oil of the present invention, are the phenyl stearates of the following metals: Aluminum, barium, cadmium, chromium, magnesium and nickel. Examples of other metallic soaps, which are useful for the purposes of my invention, are the soaps of the above-mentioned metals and other aromatic stearic acids such as, for example, tolyl stearic acid, xylyl stearic acid, naphthyl stearic acid and anthracyl stearic acid. The presence of an aromatic group in these metallic soaps seems to promote the solvent capacity of the lubricating oil composition with respect to sludge and may assist in improving its thermal stability. I have described and claimed lubricating compositions containing calcium aromatic stearates, or mixtures thereof with calcium stearate or an aromatic stearic acid, in my co-pending application Serial No. 89,120, filed July 6, 1936, which has matured into United States Patent No. 2,081,075, dated May 18, 1937.

Calcium stearate has long been used in compounded petroleum lubricating greases. This invention relates to improvements in liquid petroleum lubricants as distinguished from solid or semi-solid petroleum greases and which contain soaps of metals other than calcium. The term "petroleum lubricating oils" is intended to refer herein to lubricating oils of petroleum origin having viscosities upwards of 50-70 seconds at 100° F. Saybolt Universal.

The trend of development in internal combustion engines has imposed increasing burdens upon the oils used for their lubrication, particularly with respect to operating temperatures and pressures. At present, the Diesel type of engine probably represents extreme requirements in both of these respects, but it is not alone in the imposition of severe burdens upon the lubricating

oil used. The useful operating life of a lubricating oil, in such service, is determined, in large measure, by its thermal stability and by its physical capacity to continue functioning as a lubricant, at the high temperatures and high pressures encountered. One measure of thermal stability is resistance to oxidation, and the consequent tendency to form sludge, but in another aspect the effect of thermal instability is determined not only by the extent of oxidation or decomposition but also by the character of the products of such decomposition or oxidation and by the extent and location, within the engine, of deposits of such products.

The improved lubricating oil compositions of my invention have, in addition to the lubricating properties of the petroleum oils of which they are compounded, a high solvent capacity for sludge, of the character formed by oxidation of petroleum lubricating oils and, perhaps of even greater importance, the properties of rendering deposits of sludge and "carbon" within the engine soft and friable rather than hard and coherent and of disintegrating and removing such deposits as an incident of the normal operation of the engine. In this aspect, the lubricating oil compositions of my invention render the engines in which they are used self-cleaning to an important extent.

In the Diesel type of engine, for example, the high temperatures to which the lubricating oil is subjected, particularly at the top of the stroke, frequently causes deposition of sludge and carbonization in the groove for and behind one or more of the piston rings. Using paraffinic type lubricating oils such difficulties are usually more pronounced with respect to the uppermost ring; using naphthenic type lubricating oil they are usually more pronounced with respect to the lower rings. Consequent sticking of the rings rapidly deprives the piston and cylinder wall of proper lubrication inducing excessive wear and, frequently, scoring of the cylinder wall. The formation of such "carbon" deposits, hard enough and coherent enough to involve sticking of the rings, is materially retarded, if not avoided, by the use of the improved lubricating oil compositions of my invention, and in this aspect the self-cleaning properties of the lubricating oil compositions of my invention, with respect to the engine, make a mere change of oil a substitute, economical with respect both to loss of service time and cost, for many otherwise necessary cleaning and repair jobs.

Metallic phenyl stearates, or mixtures includ-

5

10

15

20

25

30

35

40

45

50

55

60

65

70

75

80

85

ing metallic phenyl stearates and metallic stearates, for compounding the improved lubricating oil compositions of my invention, can be produced as follows:

- 5 1 part (parts by weight) of pulverulent anhydrous aluminum chloride is stirred into 4 parts of commercial benzol boiling 90% below 100° C., this stirring being effected at atmospheric pressure and at ordinary temperature. 2 parts of 10 oleic acid, commercial red oil containing as a minimum 96% free fatty acid as oleic acid and having a maximum cloud test of 45° F., is added to this mixture with stirring, the addition being made over a period of about an hour. This re- 15 action is carried out at atmospheric pressure and is started at ordinary temperature. The temperature rise incident to the reaction is limited so that the maximum temperature approximates 180° F., the temperature being controlled either 20 by cooling or by regulating the rate of addition of the oleic acid. The reaction mixture is maintained at a temperature of 140°-180° F. for 6 or 7 hours. For at least the last half hour of this 25 period the reaction mixture is held at 180° F. to insure completion of the reaction and to assist in stripping hydrochloric acid from the reaction mixture. The reaction product, a pasty liquid, is then added to about  $\frac{1}{4}$  to  $\frac{1}{2}$  of its volume of aqueous hydrochloric acid, 15% to 20% 30 HCl, at ordinary temperature. The ensuing reaction brings the temperature, for example, to about 170° F. This reaction mixture is thoroughly stirred and the aqueous acid solution is then separated from the oily product of the re- 35 action, by decantation for example. This separated oily product is thoroughly washed with water, advantageously with hot water, in two successive stages with about  $\frac{1}{2}$  of its volume of hot water in each stage for example. This washing should in any event be continued until a 40 qualitative test for aluminum in the wash water is negative. After this washing, the reaction product is a thin, oily, dark green liquid. It is allowed to stand to settle out any remaining wa- 45 ter. Benzol is stripped from this oily liquid by distillation, limiting the maximum liquid temperature to about 350° F., using steam or other distillation medium to effect the stripping within this maximum temperature limit. The oily li- 50 quid remaining after stripping of benzol is then subjected to distillation, advantageously under a high vacuum, 2-4 millimeters of mercury absolute pressure for example. This distillation may be otherwise effected, using steam or other distillation medium for example, provided the material undergoing distillation is not heated to any temperature much exceeding 640°-650° F. for 55 any period long enough to involve decomposi- tion. When effecting the distillation under a vacuum of 4 millimeters of mercury absolute pressure, a first cut of about 25% is taken off up to the point at which the temperature of the liquid in the still reaches 466° F. and a second cut of about 53% is taken off as the temperature 60 of the liquid in the still rises from 466° F. to 590° F. The metallic phenyl stearates of the metals listed above with the exception of chromium which are used with advantage in the present invention may then be prepared from the phenyl 65 stearic acid product contained in the above-de- scribed first and second fractions, or from phenyl stearic acid or phenyl stearic acid and stearic acid mixtures obtained from other sources, as follows: 1 part of phenyl stearic acid is com- 70 pletely saponified at room temperature with the 75

theoretical quantity of 20° Bé. sodium hydroxide solution. When saponification is complete 10 parts of water are added and the mixture stirred until the sodium phenyl stearate is completely dissolved. To this solution is then added a 1:6 8 solution of a soluble salt, acetate or nitrate of the metal whose phenyl stearate is desired. This salt solution is added in sufficient excess not only to precipitate but also to coagulate the metallic phenyl stearate. The aqueous solution is de- 10 canted from the insoluble metallic soap, which is washed thoroughly with water and dried by heating on a hot plate. In the preparation of the phenyl stearic soap of chromium, the just recited procedure is followed up to the point 15 where the metallic phenyl stearate is precipitated. The nitrate or chloride is used as the precipitating agent. The further procedure is then to wash the chromium precipitate several times with water, dissolve in sufficient benzene to 20 give complete solution, filter, and remove the benzene by distillation, completing the distillation under reduced pressure.

The metallic soaps of other aromatic stearic acids may be prepared by a similar procedure. 25 The preparation of phenyl stearic acid, tolyl stearic acid and xylyl stearic acid has been described in the chemical literature (J. A. C. S. 49, 1103-1106 (1927; ibid. 52, 1172-1174 (1930)).

In referring to "metallic phenyl stearates", 30 herein, I refer to the metallic soap constituting the major portion of the product resulting from the saponification and precipitation of the second distillate fraction from the condensation of oleic acid with benzol as described above al- 35 though, of course, I intend to refer to this same material by whatever process it may be made. In referring to mixtures of "metallic phenyl stearates and metallic stearates" herein, I refer to a mixture of metallic soaps constituting the 40 major portion of the product which results if the first distillate fraction as well as the sec- 45 ond is saponified and precipitated as an insol- 50 able metal soap although, of course, I also intend to refer, by these terms, to these same materials 55 by whatever process they may be prepared. I believe the metallic phenyl stearates, referred to, to be the metallic salt of 9-, or 10-phenyl stearic acid, but I do not predicate my invention on this identification of the compound as a matter of 50 terminology. The refractive indices, acid num- 55 bers, saponification numbers and iodine numbers of the total reaction product of the oleic acid-benzol condensation, of the first and second dis- 60 tillate fractions and of the residual fraction pro- 65 duced as described in the preceding paragraph, as determined in one instance, were as follows:

|                                | Total reaction product | First cut | Second cut | Residue | 60 |
|--------------------------------|------------------------|-----------|------------|---------|----|
| Refractive index at 20° C..... | 1.4875                 | 1.4610    | 1.4880     | 1.5171  |    |
| Acid number.....               | 166                    | 193       | 155        | 127.5   |    |
| Saponification number.....     | 168.1                  | 192.6     | 160        | 161.7   |    |
| Iodine number.....             | 10                     | 1.96      | 4.08       | 23.6    | 65 |

In compounding the improved lubricating oil compositions of my invention with the usual petroleum lubricating oils, the metallic phenyl stearates, or the mixture including metallic phenyl stearates and metallic stearates, as mentioned above, are added to the lubricating oil in proportions ranging from about 0.5% up to about 2.0% or 2.5% by weight on the oil. A composition consisting chiefly of a South Texas pale oil 70

having a viscosity of 500 seconds at 100° F. Saybolt Universal and boiling approximately 10% up to 700° F. and 90% up to 900° F., and 1.3% by weight on the oil of a mixture of a phenyl stearate and a stearate of any one of the metals above described is particularly advantageous. Such a mixture of phenyl stearate and stearate is advantageously made by saponifying together the first and second distillate fractions from the vacuum distillation of the reaction mixture from the condensation of oleic acid with benzol as above described and then precipitating the desired insoluble metallic soap by adding the appropriate metal salt. The "Indiana oxidation test" on a group of compounded compositions, each containing a different one of the soaps of the recited metals, was 25-26 hours with the exception of the composition containing cadmium soap which was 22.5 hours and barium which was 16 hours. The corresponding value for the lubricating oil alone was 13.5 hours. This "Indiana oxidation test" is described in the S. A. E. Journal 34, 172-173 (1934). The same lubricating compositions, when exposed to highly heated surfaces, decompose to produce a residue consisting of a soft, friable coke in contrast to the hard and adherent residue resulting when the lubricating oil alone is so exposed. In service in a Diesel type engine these properties result in leaving the engine substantially free from sludge or carbon deposits.

The properties of these particular lubricating oils, as compared to the lubricating oil alone, as determined in one specific instance for each of the compounded mixtures using 1.33% metallic phenyl stearates prepared according to the procedure above outlined are recorded in the following table:

|                                             | South Texas oil | South Texas oil and 1.33% phenyl stearate of |             |              |
|---------------------------------------------|-----------------|----------------------------------------------|-------------|--------------|
|                                             |                 | Alum-<br>num                                 | Bar-<br>ium | Cad-<br>mium |
| Gravity.....°A. P. I.                       | 21              | 20.7                                         | 20.5        | 20.7         |
| Flash.....°F.                               | 375             | 370                                          | 375         | 385          |
| Fire.....°F.                                | 435             | 420                                          | 430         | 435          |
| Viscosity at 100° F. Saybolt Universal..... | 500             | 524                                          | 544         | 698          |
| Viscosity at 210° F.....                    | 54              | 55                                           | 55.4        | 53.2         |
| Pour.....°F.                                | -10             | -10                                          | -5          | +5           |
| Carbon residue.....                         | .048            | .133                                         | .134        | .033         |
| Ash.....percent                             | Hard            | .123                                         | .297        | .119         |
| Coke residue.....                           | Hard            | Soft                                         | Soft        | Soft         |
| Indiana sludge test.....hours               | 13.5            | 25                                           | 16          | 22.5         |

|                                             | South Texas oil | South Texas oil and 1.33% phenyl stearate of |                |        |
|---------------------------------------------|-----------------|----------------------------------------------|----------------|--------|
|                                             |                 | Chro-<br>mium                                | Magne-<br>sium | Nickel |
| Gravity.....°A. P. I.                       | 21              | 20.9                                         | 20.9           | 20.8   |
| Flash.....°F.                               | 375             | 375                                          | 375            | 370    |
| Fire.....°F.                                | 435             | 430                                          | 430            | 430    |
| Viscosity at 100° F. Saybolt Universal..... | 500             | 509                                          | 536            | 565    |
| Viscosity at 210° F.....°F.                 | 54              | 55.7                                         | 54.6           | 57.4   |
| Pour.....°F.                                | -10             | -10                                          | -10            | -10    |
| Carbon residue.....                         | .048            | .128                                         | .100           | .330   |
| Ash.....percent                             | Hard            | .077                                         | .122           | .170   |
| Coke residue.....                           | Hard            | Soft                                         | Soft           | Soft   |
| Indiana sludge test.....hours               | 13.5            | 26                                           | 25             | 25     |

The metallic phenyl stearate in each of the blends to which the foregoing table of properties relates was a substantially completely saponified metallic soap free from phenyl stearic acid, with the exception of the blend including the cadmium soap. In the case of the composition containing

the cadmium soap, the compounding agent consisted of 75% cadmium phenyl stearate and 25% free phenyl stearic acid.

Any tendency of any of the compounding agents above mentioned, abnormally to increase the viscosity of the oil to which it is added, may be reduced by the addition of a small amount of free phenyl stearic acid. In all of the above mentioned blends, with the exception of the blend including the cadmium soap, the addition of 7-8% of the acid, based on the soap, is effective for this purpose, although proportions up to about 20% are sometimes advantageous. For this purpose free stearic acid and free palmitic acid as well as mixtures of these acids alone or with phenyl stearic acid, also are useful. While the lubricating oil compositions of the foregoing examples embody specifically a South Texas lubricating oil, my invention is not limited to lubricating oil compositions embodying petroleum lubricating oil of this specific origin.

I claim:

1. A liquid lubricating oil composition comprising a petroleum lubricating oil and a metallic phenyl stearate selected from the class consisting of the phenyl stearates of aluminum, barium, cadmium, chromium, magnesium and nickel.

2. A liquid lubricating oil composition comprising a petroleum lubricating oil, a metallic phenyl stearate selected from the class consisting of the phenyl stearate of aluminum, barium, cadmium, chromium, magnesium and nickel, and a metallic stearate selected from the class consisting of the stearates of aluminum, barium, cadmium, chromium, magnesium and nickel.

3. A liquid lubricating oil composition comprising a petroleum lubricating oil, a metallic phenyl stearate selected from the class consisting of the phenyl stearates of aluminum, barium, cadmium, chromium, magnesium and nickel, and phenyl stearic acid.

4. A liquid lubricating oil composition comprising a petroleum lubricating oil, a metallic phenyl stearate selected from the class consisting of the phenyl stearates of aluminum, barium, cadmium, chromium, magnesium and nickel, a metallic stearate selected from the class consisting of the stearates of aluminum, barium, cadmium, chromium, magnesium and nickel, and phenyl stearic acid.

5. A liquid lubricating oil composition comprising a petroleum lubricating oil, a metallic phenyl stearate selected from the class consisting of the phenyl stearates of aluminum, barium, cadmium, chromium, magnesium and nickel, and stearic acid.

6. A liquid lubricating oil composition comprising a petroleum lubricating oil, a metallic phenyl stearate selected from the class consisting of the phenyl stearates of aluminum, barium, cadmium, chromium, magnesium and nickel, and a fatty acid of the class consisting of stearic acid and palmitic acid.

7. A liquid lubricating oil composition comprising a petroleum lubricating oil, a metallic phenyl stearate selected from the class consisting of the phenyl stearates of aluminum, barium, cadmium, chromium, magnesium and nickel, and a mixture of stearic acid and palmitic acid.

8. A liquid lubricating oil composition comprising a petroleum lubricating oil, a metallic phenyl stearate selected from the class consisting of the phenyl stearates of aluminum, barium, cadmium, chromium, magnesium and nickel, a metallic stearate selected from the class consisting of

ing of the stearates of aluminum, barium, cadmium, chromium, magnesium and nickel, and stearic acid.

9. A liquid lubricating oil composition comprising a petroleum lubricating oil, a metallic phenyl stearate selected from the class consisting of the phenyl stearates of aluminum, barium, cadmium, chromium, magnesium and nickel, a metallic stearate selected from the class consisting of the 10 stearates of aluminum, barium, cadmium, chromium, magnesium and nickel, and a fatty acid of the class consisting of stearic acid and palmitic acid.

10. A liquid lubricating oil composition comprising a petroleum lubricating oil and a metallic aromatic stearate selected from the class consisting of the aromatic stearates of aluminum, barium, cadmium, chromium, magnesium and nickel.

11. A liquid lubricating oil composition comprising a petroleum lubricating oil, a metallic aromatic stearate selected from the class consisting of the aromatic stearates of aluminum, barium, cadmium, chromium, magnesium and nickel, and an aromatic stearic acid.

12. A liquid lubricating oil composition comprising a petroleum lubricating oil, a metallic aromatic stearate selected from the class consisting of the aromatic stearates of aluminum, barium, cadmium, chromium, magnesium and nickel, and a fatty acid of the class consisting of stearic acid and palmitic acid.

13. A liquid lubricating oil composition comprising a petroleum lubricating oil, a metallic aromatic stearate selected from the class consisting of the aromatic stearates of aluminum, barium, cadmium, chromium, magnesium, and nickel, and a mixture of stearic acid and palmitic acid.

14. A liquid lubricating oil composition comprising a petroleum lubricating oil and magnesium phenyl stearate.

15. A liquid lubricating oil composition comprising a petroleum lubricating oil and chromium phenyl stearate.

16. A liquid lubricating oil composition comprising a petroleum lubricating oil and aluminum phenyl stearate.

ARNOLD C. VOBACH.